

# UNITED STATES PATENT OFFICE.

LOUIS S. ROSS, OF NEWTONVILLE, MASSACHUSETTS.

## TIME-BURNING RAILWAY SIGNAL-FUSEE.

1,059,768.

Specification of Letters Patent. Patented Apr. 22, 1913.

No Drawing.

Application filed November 16, 1912. Serial No. 731,907.

To all whom it may concern:

Be it known that I, LOUIS S. ROSS, a citizen of the United States, and a resident of Newtonville, in the county of Middlesex and 5 State of Massachusetts, have invented an Improvement in Time-Burning Railway Signal-Fusees, of which the following description is a specification.

This invention relates to improvement in 10 time burning railway signal fusees, the primary object thereof being to produce a fusee for such purpose that will not spontaneously ignite under conditions to which it is necessarily subjected, which will not be 15 extinguished when thrown from a moving train or otherwise subjected to severe shock, but which is very inflammable, easily ignited, and insures continuity of the flame after lighting, and which is not subject to 20 certain defects that have previously characterized the so-called perchlorate fusee.

A fusee made of mixtures containing a perchlorate, such as perchlorate of potassium, is recognized to be harder to ignite 25 and more easily extinguished when thrown from a moving train than a fusee of the so-called chlorate type. The so-called perchlorate fusee, in spite of this objection, is used because of its substantial freedom from 30 spontaneous ignition. Not only is the so-called perchlorate fusee objectionable because it is more readily extinguished when thrown, but also because it burns with a greater brilliancy tending toward incandescence; it possesses a decreased burning 35 interval, and it is necessarily manufactured at a greater cost.

The greater brilliancy of the perchlorate fusee is caused by the increased oxidizing 40 power of the chemicals required. This disadvantage becomes most serious where the fusees burn with combination colors for the tendency to incandescence and excessive brilliancy causes the red, yellow and green 45 fusee flames to lose their characteristic colors and gradually merge nearer a white light.

In all fusees there is a period known as the quickening up of the fusee, by which is meant the tendency to burn a shorter 50 time than when first made. This is particularly noticeable in the perchlorate fusee, as such perchlorate fusee must be made with a longer burning interval when new, in order to prevent the possibility of burning 55 under time at the end of a few months.

To overcome this disadvantage increased length of case is necessary, which is a further disadvantage because the longer the fusee, the more leverage is possessed by the fusee when thrown from the train, with 60 the resultant increased tendency toward breaking.

The greater cost of perchlorate, such, for example, as perchlorate of potassium over chlorate of potassium, is also a serious objection to the so-called perchlorate fusee. Because of the fact that a perchlorate fusee is substantially free from danger of spontaneous ignition, although open to other objections, some of which I have above enumerated, I have conducted a series of experiments in order to produce if possible a fusee having a minimum quantity or proportion of perchlorate, as, for example, perchlorate of potassium, thereby reducing 70 or overcoming the objections to which the so-called perchlorate fusee is subject, while possessing freedom from spontaneous ignition. In other words, I have endeavored to produce a fusee having freedom from spontaneous ignition and yet not readily extinguished by shock when thrown, which does not burn with a brilliancy tending toward incandescence, but which burns with greater inflammability than the so-called perchlorate fusee and with a lower temperature of ignition, without possessing the decreased burning interval of the perchlorate fusee and the increased cost of the latter. I have as the result of said experiments discovered that excellent results may be obtained by employing perchlorate such, for 80 example, as perchlorate of potassium, barium, sodium or ammonium, together with at least as great or a greater quantity of 85 chlorate, such, for example, as chlorate of potassium, of barium, of sodium, of ammonium or any other suitable chlorate. I have discovered that the temperature of ignition of the fusee decreases as the quantity of chlorate increases, but that the lower 90 the temperature of ignition of the fusee, the more force of flame and the greater inflammability of the fusee. A lower temperature of ignition of the fusee is desirable, provided it be free from tendency to spontaneous ignition, as a fusee possessing such characteristic will, when nearly extinguished, revive and burn, due to the lower 95 temperature required for rekindling. Fur- 100

105 110

thermore, the greater the quantity of chlorate, the more inflammable is the fusee and the more easily is it ignited.

As the result of my experiments, I have discovered that it is not necessary entirely to replace the chlorate of the old so-called chlorate fusee by perchlorate, as had been supposed, nor is it necessary to use a relatively large quantity of perchlorate of potassium when compared with the quantity of chlorate of potassium. On the other hand, the results of my experiments have distinctly shown that I may very largely reduce the quantity or proportion of perchlorate and employ a quantity of chlorate, at least as great as the quantity of perchlorate and preferably greater. The resulting fusee is not liable to spontaneous ignition and it is of increased inflammability compared with the so-called perchlorate fusee, while the tenacity and force of the fusee composition are increased. Moreover, the fusee is not readily extinguished under adverse conditions and the fusee is not as readily extinguished by sudden shock by being thrown from a train as is the so-called perchlorate fusee.

Perchlorate fusees as heretofore manufactured usually contain from five or six to twenty per cent. of potassium or other perchlorate, combined with which are nitrate, sulfur and carbohydrate, with charcoal and antimony if desired, in substantially the following proportions:—nitrate 50 to 95%, sulfur 3 to 23%, carbohydrate 1 to 11%, charcoal 1%, antimony 1%.

In accordance with my invention, I preferably provide as customary in the so-called perchlorate fusee, sulfur, hydrocarbon, carbohydrate or other suitable carbonaceous material, and a metallic salt, such as a metallic nitrate or oxid, to which, if desired, I may add charcoal and antimony. The sulfur is mainly used to increase combustion, the hydrocarbon and the carbohydrate or carbonaceous material are used to furnish carbon and hydrogen to aid combustion and to smooth and deepen the flame, and the metallic salt, which is preferably that of strontium, barium or sodium, constitutes the base or color ingredient. In other words the metallic salt employed burns with oxidation and a colored flame. To this or other desired ingredients, I add a suitable quantity of perchlorate (preferably perchlorate of potassium) though I may employ any suitable perchlorate, such, for example, as barium, sodium or ammonium perchlorate, and at least as great and preferably a greater quantity of chlorate (preferably chlorate of potassium, though I may employ any suitable chlorate, such for example as chlorate of barium, of sodium or of ammonium).

While the proportions of the several ingredients may be varied, they may be those

stated for nitrate, sulfur, carbonaceous material, and antimony if desired, with the hereinafter described admixture of perchlorate and of chlorate.

The carbonaceous material preferably employed by me consists of rosin or red gum, charcoal and sawdust and grease in suitable proportions. The red gum employed is the powdered bark of the red gum (*Eucalyptus rostrata*). It will be understood that I may employ one or more carbohydrates, hydrocarbons or carbons, either alone or in any suitable mixture, or that any two of such carbonaceous materials may be employed. I have obtained excellent results by employing the following formula wherein the ingredients are specified in percentages:—metallic nitrate 50 to 80%, sulfur 10 to 15%, carbohydrate 2 to 7%, hydrocarbon 1 to 3%, perchlorate of potassium, of barium, of sodium or of ammonium 2½ to 10%, chlorate of potassium, of barium, of sodium or of ammonium 2½ to 19%.

I set forth definitely a specific formula in the use of which I have obtained excellent results, as follows:—metallic nitrate 61%, sulfur 12%, carbohydrate 5%, hydrocarbon 2%, perchlorate of potassium 8%, chlorate of potassium 12%.

In any case the quantity of chlorate used at least equals the quantity of perchlorate used, and if the quantity of perchlorate is decreased, then preferably the quantity of chlorate is correspondingly increased, so that the sum of the quantities of chlorate and perchlorate remains the same, thus reducing cost and insuring reliability.

By largely reducing the quantity of perchlorate, I have, as previously stated, removed the objections incident to the so-called perchlorate fusee, and I have succeeded in obtaining a fusee which is not subject to spontaneous ignition or combustion.

Although the fusee obtained by me is not subject to spontaneous combustion, I may, if desired, employ a so-called ant-acid or neutralizing agent, preferably calcium or other carbonate, which will neutralize any possible tendency to an acid re-action of the sulfur and chlorate of potassium, while not impairing the brilliancy and the force of flame. Such neutralizing agent, if employed, does not constitute a greater proportion than one half to three per cent. of the entire composition.

The fusee constructed in accordance with my invention burns with tenacity and force, and the temperature of ignition is not maintained at such a height as to render difficult the reviving or re-kindling of the fusee when nearly extinguished from shock or other cause.

Preferably, I employ potassium chlorate in a red fusee and barium chlorate in a green fusee, but by using any chlorate, I have suc-

ceeded in making a railway time burning signal fusee having all the advantages of the chlorate fusee, and yet not possessing the characteristic disadvantages of the so-called perchlorate fusee previously pointed out.

The time burning railway signal fusee compound embodying my invention contains as essential ingredients a perchlorate and a chlorate in the proportions herein set forth, it being noted that the chlorate is equal to or greater in quantity than the perchlorate, any suitable perchlorate and any suitable chlorate being used, together with sulfur. To this composition, I add one or more of the other ingredients specified by me, and for the best results I add metallic nitrate and some suitable carbonaceous material.

I employ the term "carbonaceous material" to include hydrocarbon, carbohydrate, carbons and other suitable carbon containing material.

I may employ any suitable metallic salt in the production of the fusee, of which a metallic nitrate is an example.

Having thus described one embodiment of my invention and the best manner known to me for carrying the same into effect, I desire it to be understood that the scope of the invention is set forth in the following claims.

Claims:

1. A time burning railway signal fusee comprising a metallic nitrate, carbonaceous material, sulfur, perchlorate, and a quantity of chlorate at least equaling the quantity of perchlorate, thereby producing a time burning railway signal fusee compound burning with brilliancy, marked inflammability, tenacity and force of flame and not liable to spontaneous ignition or combustion, nor readily extinguished by shock.

2. A time burning railway signal fusee including a metallic salt burning with oxidation and a colored flame, sulfur, perchlorate, and a quantity of chlorate at least equaling the quantity of perchlorate, thereby producing a time burning railway signal fusee compound burning with brilliancy, marked inflammability, tenacity and force of flame and not liable to spontaneous ignition or combustion nor readily extinguished by shock.

3. A time burning railway signal fusee including sulfur, metallic nitrate, perchlorate, and a quantity of chlorate at least equaling the quantity of perchlorate, thereby producing a time burning railway signal fusee compound burning with brilliancy, marked inflammability, tenacity and force of flame and not liable to spontaneous ignition or combustion nor readily extinguished by shock.

4. A time burning railway signal fusee comprising a metallic nitrate, carbonaceous

material, sulfur, perchlorate of potassium, and a quantity of chlorate of potassium at least equaling the quantity of perchlorate of potassium, thereby producing a time burning railway signal fusee compound burning with brilliancy, marked inflammability, tenacity and force of flame and not liable to spontaneous ignition or combustion nor readily extinguished by shock.

5. A time burning railway signal fusee comprising a metallic salt, burning with oxidation and a colored flame, sulfur, hydrocarbon, carbon, perchlorate of potassium, and a quantity of chlorate of potassium at least equaling the quantity of perchlorate of potassium, thereby producing a time burning railway signal fusee compound burning with brilliancy, marked inflammability, tenacity and force of flame and not liable to spontaneous ignition or combustion nor readily extinguished by shock.

6. A time burning railway signal fusee comprising fifty to eighty per cent. metallic nitrate, ten to fifteen per cent. sulfur, three to ten per cent. carbonaceous material, two and a half to ten per cent. perchlorate of potassium, two and a half to nineteen per cent. chlorate of potassium, but the percentage of chlorate at least equaling that of the perchlorate, thereby producing a time burning railway signal fusee compound burning with brilliancy, marked inflammability, tenacity and force of flame and not liable to spontaneous ignition or combustion nor readily extinguished by shock.

7. A time burning railway signal fusee comprising fifty to eighty per cent. metallic nitrate, ten to fifteen per cent. sulfur, three to ten per cent. carbonaceous material, two and a half to ten per cent. perchlorate of potassium, and a quantity of chlorate of potassium substantially greater than the quantity of perchlorate of potassium, thereby producing a time burning railway signal fusee compound burning with brilliancy, marked inflammability, tenacity and force of flame and not liable to spontaneous ignition or combustion nor readily extinguished by shock.

8. A time burning railway signal fusee comprising a metallic nitrate, sulfur, a chlorate, and a quantity of perchlorate smaller than the quantity of chlorate, thereby producing a time burning railway signal fusee compound burning with brilliancy, marked inflammability, tenacity and force of flame and not liable to spontaneous ignition or combustion nor readily extinguished by shock.

9. A time burning railway signal fusee comprising a metallic nitrate, carbonaceous material, sulfur, perchlorate of potassium, a quantity of chlorate of potassium at least equaling the quantity of perchlorate of potassium, and an acid neutralizing agent,

4  
thereby producing a time burning railway signal fusee compound burning with brilliancy, marked inflammability, tenacity and force of flame and not liable to spontaneous ignition or combustion nor readily extinguished by shock.

10. A time burning railway signal fusee comprising a metallic nitrate, carbonaceous material, sulfur, perchlorate of potassium, a quantity of chlorate of potassium at least equaling the quantity of perchlorate of potassium, and a small quantity of calcium carbonate, thereby producing a time burning railway signal fusee compound burning with brilliancy, marked inflammability, tenacity and force of flame and not liable to spontaneous ignition or combustion nor readily extinguished by shock.
15. A time burning railway signal fusee

comprising about sixty-one per cent. metallic nitrate, twelve per cent. sulfur, five per cent. carbohydrate, two per cent. hydrocarbon, eight per cent. perchlorate of potassium, twelve per cent. chlorate of potassium, thereby providing a time burning railway signal fusee compound burning with brilliancy, marked inflammability, tenacity and force of flame and not liable to spontaneous ignition or combustion nor readily extinguished by shock.

30  
In testimony whereof, I have signed my name to this specification, in the presence of two subscribing witnesses.

LOUIS S. ROSS.

Witnesses:

IRVING U. TOWNSEND,  
ROBERT H. KAMMLER.